

# UNITED STATES PATENT OFFICE.

MAX CLINE AND CHARLES F. RHODES, OF GLENS FALLS, NEW YORK, ASSIGNEES TO  
INTERNATIONAL PAPER COMPANY, OF NEW YORK, N. Y., A CORPORATION OF NEW  
YORK.

## METHOD OF REMOVING INK FROM PAPER-STOCK.

1,138,085.

Specification of Letters Patent.

Patented May 4, 1915.

No Drawing.

Application filed November 27, 1911. Serial No. 662,579.

*To all whom it may concern:*

Be it known that we, MAX CLINE and CHARLES F. RHODES, citizens of the United States, residing at Glens Falls, county of 5 Warren, State of New York, have invented certain new and useful Improvements in Methods of Removing Ink from Paper-Stock; and we do hereby declare the following to be a full, clear, and exact description 10 of the invention, such as will enable others skilled in the art to which it appertains to make and use the same.

This invention relates to a certain new and useful improvement in the removal of 15 printers' ink from old paper stock, that is to say from stock made up in whole or in part of waste printed paper, as, for instance, from old newspapers, printed books, and the like.

20 In the practice of the invention, the waste paper stock is macerated in the presence of water in a beater engine or any machine for reducing it to a substantially homogeneous pulp. To the original or macerated stock, 25 containing the ink to be removed, is added a caustic alkali, in solution, preferably caustic soda, which has the effect of "lifting" the ink from the fiber. There is also added to the original or macerated stock a 30 quantity of silicate of aluminum such as fullers' earth, kaolin and all other clays or silicate of magnesium such as talc, soapstone, etc., which serve to take up, absorb, or carry the ink, thereby segregating it from the fiber. Finally, by a washing operation, 35 the aluminum silicate or clays, carrying with it the ink, is separated from the fiber, thereby bringing the stock back quite closely to the original condition and color of raw stock.

40 As an illustration of the successful practice of the invention, it may be stated that successful results may be obtained by first macerating the waste printed paper stock or book stock with the necessary amount of water to bring it to a pulp. This operation can be carried on in a beater engine or in any other suitable type of pulping machine, and with water at ordinary atmospheric temperatures. To the macerated or pulped 45 stock is then added the caustic alkali and the absorbing agent, in the proportion of,

say, forty pounds of caustic soda (sodium hydrate), and forty pounds of aluminum silicate or clay, per ton of the pulped stock of beater consistency. The caustic alkali 55 thereupon exercises its function of lifting the ink from the fiber of the stock and the aluminum silicate or clay is found to absorb, take up, and carry the ink, thereby segregating it from the fiber. The operation is 60 facilitated and made uniform by vigorously agitating and mixing the mass for a period varying from say ten minutes to thirty minutes according to the character of the stock employed and the desired completeness 65 of the result. In some instances, also, it may be further facilitated by raising the temperature of the stock by the injection of steam or the addition of hot water. Thereupon the aluminum silicate or clay, carrying the ink, 70 is washed from the fiber in any suitable manner, as, for instance, in the drum washer in common use in paper mills, in which also the stock may be macerated, treated and washed, or by any other washing method 75 desirable.

What we claim is:

1. The process of removing ink from waste newspaper stock, book stock, and the like, which consists in pulping the stock, 80 adding a caustic alkali thereto for lifting the ink, adding aluminum silicate or clay, to absorb the lifted ink, and washing out the ink-carrying absorbent; substantially as described.

85 2. The process of removing ink from waste newspaper stock, book stock, and the like, which consists in pulping the stock, lifting the ink by adding about 2% of caustic soda, absorbing the lifted ink by adding about 2% of aluminum silicates such as fullers' earth, kaolin and other clays, or magnesium silicates such as talc, soapstone, etc., and washing out the ink-carrying absorbent; substantially as described. 90 95

In testimony whereof we affix our signatures, in presence of two witnesses.

MAX CLINE.

CHARLES F. RHODES.

Witnesses:

EDWARD J. TRIMBEY,  
KATHERINE E. BUSWELL.